

Dec. 28, 1948.

A. J. MILLER ET AL

2,457,169

METHOD OF MANUFACTURING OF RECTIFIER ELEMENTS

Filed March 12, 1945

2 Sheets-Sheet 1

BLOCKING  
ABILITY  
AND  
ELECTROFORMING  
RATE

Fig. 1.



FORWARD  
CONDUC-  
TIVITY

Fig. 2.



INVENTORS  
ARTHUR J. MILLER  
JULIUS W. FLEISHER

BY

*Marshall Rosenbaum, Jr.*  
ATTORNEY

Dec. 28, 1948.

A. J. MILLER ET AL

**2,457,169**

## METHOD OF MANUFACTURING OF RECTIFIER ELEMENTS

Filed March 12, 1945

2 Sheets-Sheet 2



BY

**INVENTORS**  
**ARTHUR J. MILLER**  
**JULIUS W. FLEISHER**

ATTORNEY

## UNITED STATES PATENT OFFICE

2,457,169

METHOD OF MANUFACTURING OF  
RECTIFIER ELEMENTS

Arthur J. Miller, Oak Ridge, Tenn., and Julius W. Fleisher, New York, N. Y., assignors to Federal Telephone and Radio Corporation, New York, N. Y., a corporation of Delaware

Application March 12, 1945, Serial No. 582,278

5 Claims. (Cl. 175—366)

1

This invention relates to a method of manufacturing of rectifier elements and to the rectifier element itself, and has for its main object to provide rectifier elements particularly selenium elements which have a better blocking layer than the elements manufactured according to previously used methods.

In the manufacture of selenium elements in a well known manner a coating of selenium is provided on a base plate and the selenium layer is annealed by heat treatment to crystallize the selenium. This annealing process is ordinarily done in two heat treatment steps: the first step involves heating the selenium to 120° C. under pressure for about one-half hour; and the second step involves heating without pressure for several hours at a higher temperature just under the melting point of selenium, for example, about 214° C. A treatment is then usually given the selenium with selenium dioxide vapor or selenium vapor after which a conducting counter-electrode is sprayed over the selenium surface.

It has been found that the final treatment of the selenium with selenium vapor is preferable to the treatment with selenium dioxide vapor since the first mentioned treatment provides a better blocking layer than the later mentioned one. In many cases, however, the blocking layer thus achieved was still not yet satisfactory and according to the method of the present invention it is possible to provide a still more improved blocking layer.

It is, therefore, the main object to provide a method for manufacturing of selenium elements which have a better blocking layer and electro-forming rate than achieved before by using known methods.

It is a further object of the present invention to provide a method for manufacturing of selenium elements which have a better forward conductivity though the blocking and electroforming rate are improved.

It is still another object of the present invention to provide a selenium element which has improved blocking layer characteristics, electro-forming rate and forward conductivity.

With these and other objects in view which will become apparent in the following description, the invention will be clearly understood in connection with the enclosed drawings, in which:

Figure 1 shows a diagram of heat treatment temperature against blocking ability and electro-forming rate;

Fig. 2 shows a diagram of heat treatment temperature against forward conductivity; and

2

Fig. 3 shows a schematic elevational view of an apparatus for performing the method according to the present invention.

It has been found that by providing a third heat treatment, instead of selenium vapor treatment or selenium dioxide vapor treatment, at a temperature between 300 to 450° C. for two or three seconds, an improved blocking layer compared with that achieved before by the selenium vapor treatment is provided.

In Figure 1 it is clearly shown that the lowest blocking ability and electroforming rate is achieved when the manufacturing process is stopped after the second heat treatment of the selenium. If a selenium dioxide vapor treatment is used the blocking layer is quite improved, yet the best results achieved heretofore were obtained by the selenium vapor treatment. The curve shown in Figure 1 in full lines discloses clearly that by providing a third heat treatment within the temperature range of 300 to 450° C. a still better blocking layer can be achieved than that obtained by selenium vapor treatment.

Fig. 2 discloses clearly that the best forward conductivity is achieved when the manufacturing process is stopped after the second heat treatment. If the second heat treatment is followed by selenium dioxide treatment the forward conductivity is lowered tremendously. Quite an improvement can be achieved by providing a selenium vapor treatment instead of a selenium dioxide vapor treatment, yet, as Fig. 2 shows clearly again, the forward conductivity receives still a set back compared with that prevailing after the second heat treatment.

It has been found that the provision of the above described third heat treatment particularly in the temperature range of 300 to 450° C. also improves the forward conductivity compared with that achieved by selenium vapor treatment and is substantially equal to the forward conductivity prevailing after the second heat treatment.

Fig. 3 shows, by example only, an apparatus which can be used to perform the method according to the present invention. It is emphasized, however, that the apparatus per se as shown cannot be considered as limitation of the present invention. As shown in Fig. 3 a plurality of base plates 1 having a selenium layer 2 applied under pressure during the first heat treatment process may be moved on an endless belt 3, an oven 4 to be exposed to the second heat treatment and finally through another oven 5, to be exposed to the third heat treatment. The oven 5 is heated

up for example by a heating coil 6 and pipes (not shown) can be inserted into the oven chamber 5 to introduce CO<sub>2</sub> when the performance in a CO<sub>2</sub> atmosphere is preferred.

From the above stated findings can be concluded that the substitution of the selenium dioxide vapor treatment or of the selenium vapor treatment by a third heat treatment particularly in the above mentioned temperature range not only improves the blocking ability and electro-forming rate of the selenium element but at the same time improves the forward conductivity, thus resulting in an improvement of several characteristics of the selenium rectifier element.

It has been further found that more beneficial results are achieved when the third heat treatment takes place in a CO<sub>2</sub> atmosphere.

By using the method according to the present invention it is possible to eliminate all the fuming and handling by placing a thin strip heater above the conveyor to third heat treat the discs after they leave the second heat treatment oven.

While we have disclosed the principle of our invention in connection with one embodiment and a modification thereof, it will be understood that these embodiments are given by way of example only and not as limiting the scope of the invention as set forth in the objects and appended claims.

What we claim is:

1. The method of manufacturing a selenium rectifier element which comprises applying a first heat treatment of selenium to about 120° C. under pressure, then after cooling off the selenium layer applying a second heat treatment without pressure at a higher temperature than that applied in the first heat treatment yet below the melting point of the selenium, and after cooling the selenium to about room temperature applying a momentary third heat treatment at a temperature ranging from 300 to 450° C. 40

2. The method of manufacturing a selenium rectifier element, as set forth in claim 1, the said third heat treatment being applied for two or three seconds.

3. The method as set forth in claim 1, com-

prising applying the said third heat treatment for a period of two or three seconds in a CO<sub>2</sub> atmosphere.

5. A selenium rectifier element comprising a base plate having a selenium layer, said layer having been exposed to a first heat treatment at about 120° C. under pressure, a second heat treatment without pressure at a higher temperature than that applied in the first heat treatment yet 10 below the melting point of selenium and a momentary third heat treatment, the third heat treatment being at a temperature range between 300 and 450° C., the selenium layer being cooled between the first and second heat treatments and between the second and third heat treatments.

6. A selenium rectifier element comprising a base plate having a selenium layer, said layer having been exposed to a first heat treatment at about 120° C., under pressure, a second heat treatment without pressure at a higher temperature than that applied in the first heat treatment yet below the melting point of selenium and a momentary third heat treatment, the third heat treatment being at a temperature range between 20 300 and 450° C. in a CO<sub>2</sub> atmosphere, the selenium layer being cooled between the first and second heat treatments and between the second and third heat treatments.

ARTHUR J. MILLER.  
JULIUS W. FLEISHER.

#### REFERENCES CITED

The following references are of record in the file of this patent:

#### UNITED STATES PATENTS

| Number       | Name         | Date           |
|--------------|--------------|----------------|
| 1,743,160    | Presser      | Jan. 14, 1930  |
| 2,193,610    | Wilson       | Mar. 12, 1940  |
| 2,215,999    | Brunke       | Sept. 24, 1940 |
| 2,226,716    | Geisler      | Dec. 31, 1940  |
| 2,279,187    | Thompson     | Apr. 7, 1942   |
| 2,356,094    | Saslaw       | Aug. 15, 1944  |
| 2,363,555    | Saslaw       | Nov. 28, 1944  |
| 45 2,395,259 | Ellis et al. | Feb. 19, 1946  |